

## UNITED STATES PATENT OFFICE

2,215,442

## ALUMINUM ALLOY AS BEARING METAL

Eugen Vaders, Frankfort-on-the-Main, Germany,  
assignor to Vereinigte Deutsche Metallwerke  
Aktiengesellschaft, Frankfort-on-the-Main-  
Heddernheim, Germany

No Drawing. Original application December 15,  
1937, Serial No. 180,029. Divided and this ap-  
plication December 26, 1939, Serial No. 311,057.  
In Germany December 16, 1936

4 Claims. (Cl. 75—148)

In the white metal bearings heretofore com-  
monly used the base metal consists principally of  
tin or of lead. The tin generally contains addi-  
tions of antimony, bismuth, copper, etc., where-  
as the lead is alloyed principally with antimony  
and bismuth. The bearing metals having a tin  
base have up to now been considered the best of  
their kind. But in consequence of their high tin  
content which amounts up to 90%, they are very  
expensive so that for the sake of economy the  
expensive tin has been replaced by the cheaper  
lead. The lead content is very often used in the  
same proportion as the tin in the tin bearing  
metals. Even the additions are very often the  
same.

Since, according to views very often held, such  
metal alloys are best suited for bearing purposes  
in which the structure is composed of various  
hard components, it should be theoretically pos-  
sible to use every metal as base metal for a bear-  
ing metal alloy, provided that other metals ex-  
ist, which when added to this base metal alloy,  
form hard compounds with it. Aluminum is  
known to form numerous compounds with other  
metals and it has been proposed to use alumini-  
num alloys for bearing purposes. This has, on  
several occasions, been tried but with very little  
success considering the fact that most aluminum  
bearing metals of the type referred to contain  
hard compounds which wear the axle too much.  
Bearing metals of this kind are, e. g., the alumini-  
num-silicon-alloys with high silicon content or  
aluminum-magnesium-silicon-alloys.

According to the present invention much more  
useful aluminum alloys result from the addition  
of metals which form with the aluminum none or  
at least only few hard compounds, thus resulting  
in no damage being done to the axle even after  
an extended time of working. Such additions  
are antimony and lead which may be present in  
quantities up to 10% each. The antimony forms  
with aluminum the compound AlSb which is  
present in the base alloys as bearing component.  
Lead does not combine with aluminum. Ac-  
cording to the opinion of several experts it is  
not soluble at all in the aluminum. If aluminum  
be melted together with lead, at the time of solid-  
ification a separation of the aluminum and lead  
takes place i. e. the lead is as insoluble in the  
aluminum as oil in water. By adding antimony  
to the aluminum this sharp separation of lead  
from the aluminum is obviated, so that with the  
presence of a sufficient quantity of antimony  
larger quantities of lead are distributed in the  
aluminum, resulting in an alloy which shows a

structure more especially suitable for bearing  
purposes. Apart from aluminum an AlSb com-  
pound is contained in it, while lead is either al-  
loyed with this Al-Sb compound, or else is segre-  
gated in form of small drops which form an im-  
provement of the sliding surface, inasmuch as in  
the case of interruption of the oiling or sudden  
stoppage of the running of the bearing no damage  
will be caused to the axle. All tests made in this  
direction proved in every instance that the slid-  
ing surface of the axle was covered with a thin  
layer of the aluminum alloy, that could easily be  
removed. The aluminum-antimony-lead-alloys  
have a crystalline structure as also the other  
qualities of the known white bearing metal. 15  
Thus they are easily formable even in a cold state.

The sliding properties have been ascertained  
with an especially suitably alloy consisting of  
2.5% Pb, 2.5% Sb and the balance aluminum by  
a bearing testing installation. On that occasion 20  
specific surface pressures of about 200 kg./cm.<sup>2</sup>  
could be reached at a speed of 10 m./sec., where-  
by the bearing temperature rose up to 100° C.  
The test axle that consisted of non-hardened  
steel was perfectly smooth and free from indent 25  
at the end of the test. Apart from the bearing  
testing machine, tests were made in combustion  
motors in which the connecting rod bearings con-  
sisted of the new aluminum alloys. These com-  
bustion motors have been driven by an electrical 30  
motor, so that the bearings were fully charged.  
Also in that case the bearings of the new alloy  
proved successful, for during a working period of  
about 6 weeks the motors did not show any de-  
fects.

On further investigation of these alloys it was  
shown that the lead and the antimony can be  
replaced in part at least by one of the metals of  
the group tin, cadmium, calcium and arsenic in  
quantities of 0.1-5%. Thus it is possible to make 40  
use with equal success of an alloy of the follow-  
ing composition:

|    | Percent |
|----|---------|
| Pb | 1.5     |
| Sn | 1       |
| Sb | 2.5     |
| Al | Balance |
| or |         |
| Pb | 2.5     |
| Sn | 1       |
| Sb | 1.5     |
| Al | Balance |

In cases in which the price of the bearing metal 55

is of lesser importance, the tin content may also be higher. An alloy having a higher tin content is about the following:

|      | Percent |
|------|---------|
| 5 Pb | 2.5     |
| Sb   | 2.3     |
| Sn   | 5       |
| Al   | Balance |

10 Since tin alloys well either with antimony or with lead, it is particularly valuable as addition to the ternary aluminum-lead-antimony-alloy, but also the other metals added to this three-part-alloy result in very useful bearing metals.

15 While the additional metals mentioned above influence chiefly the sliding properties, the further possible additions of at least one of the metals of the group consisting of copper, nickel, cobalt, iron, manganese and zinc in quantities of

20 0.1-10% and silicon in quantities of 0.1-3% especially effect a strengthening of the bearing metal which consequently is more suitable to resist higher pressures. Especially an addition of manganese has proved very effective, inasmuch as it not only increases the hardness of the alloy, but even improves essentially the sliding properties. An alloy that proved particularly useful for the automobile motor is composed as follows: 2.5% Pb, 2.5% Sb, 3% Mn, remainder Al.

25 30 Further alloys that correspond about with the properties of the above mentioned alloys are as follows:

|       | Percent  |   |   |   |   |   |   |   |   |   |   |   |   |     |     |     |     |
|-------|----------|---|---|---|---|---|---|---|---|---|---|---|---|-----|-----|-----|-----|
|       | Pb       | 3 | 3 | 3 | 3 | 3 | 5 | 4 | 3 | 5 | 3 | 3 | 3 | 5   | 7   | 8   | 1   |
| 35 Sb | 3        | 3 | 3 | 3 | 3 | 3 | 4 | 5 | 5 | 3 | 3 | 3 | 3 | 6   | 6   | 7   | 8   |
| Sn    | 3        | 3 | 3 | 3 | 3 | 3 | 5 | 2 | 5 | 5 | 2 | 2 | 2 | 3   | 3   | 3   | 3   |
| Cd    | 3        | 3 | 3 | 3 | 3 | 3 | 5 | 2 | 5 | 5 | 2 | 1 | 1 | 1   | 2   | 3   | 3   |
| As    |          |   |   |   |   |   |   |   |   |   |   |   |   | 0.5 | 0.5 | 0.5 | 0.5 |
| Mn    |          |   |   |   |   |   |   |   |   |   |   |   |   | 3   | 3   | 3   | 3   |
| 40 Ni |          |   |   |   |   |   |   |   |   |   |   |   |   | 2   | 1   | 2   | 2   |
| Co    |          |   |   |   |   |   |   |   |   |   |   |   |   | 3   | 3   | 3   | 3   |
| Cu    |          |   |   |   |   |   |   |   |   |   |   |   |   | 0.5 | 0.5 | 0.5 | 0.5 |
| Fe    |          |   |   |   |   |   |   |   |   |   |   |   |   | 1   | 1   | 1   | 1   |
| Zn    |          |   |   |   |   |   |   |   |   |   |   |   |   | 2   | 2   | 2   | 2   |
| Si    |          |   |   |   |   |   |   |   |   |   |   |   |   | 0.3 | 0.3 | 0.3 | 0.3 |
| 45 Al | Balance. |   |   |   |   |   |   |   |   |   |   |   |   |     |     |     |     |

The addition of metals of a higher melting point further serve the purpose of making the bearing metals capable of resisting higher temperatures. While it is correct that with most of the additional metals named above the melting point of aluminum is lowered to the eutectic point, the presence of these metals having higher melting points, more especially if lead and tin with their lower melting point are present, result in the direction of a better resistance to higher temperatures. Bearing temperatures of up to 120° C. could be reached without a clinging or sticking to the axle having occurred. Naturally with such high temperatures the higher heat expansion of the aluminum alloys has to be taken into

account by the provision of a greater bearing-play.

If the new bearing metals are used under favorable conditions, i. e., presence of ample quantities of lubricants, they show but a small wear, even after a comparatively short running-in period.

Summing up it may be said that with the new bearing metals having an aluminum base as compared with the hitherto known bearing metals, the following advantages exist:

1. Easier running-in,
2. High resistance to wear,
3. Possibility to use unhardened axles,
4. High resistance to temperature.

The alloys may be used in accordance with the invention for any casting method, as sand casting, chill casting, pressure die casting and centrifugal casting. With centrifugal casting the temperatures and numbers of revolutions must be adjusted in such a way that the segregations remain at a minimum. The alloys may further be pressed, forged or rolled. In this respect it is surprising that the annealing in the drawing of rods and tubes may be accomplished at about 500° C. in spite of the lead and antimony content without a segregation of the alloys occurring thereby.

For the production of an alloy as uniform as possible, first of all antimony is melted together with aluminum whereupon lead is added as such or as a preliminary alloy.

The rolling possibility moreover makes it possible to roll up the alloys to a firmer sheet base that may consist of iron or copper alloys or also of hardenable aluminum alloys and to produce from the compound metal sheets thus obtained especially firm bearing shells.

This application is a division of my copending application, Serial No. 180,029, filed December 15, 1937, now Patent No. 2,196,236, patented April 9, 1940.

I claim:

1. A bearing metal alloy containing about 1-10% of lead, 1-10% of antimony, 0.1-3% of silicon, and 0.1-10% of a metal of the group consisting of nickel, cobalt and iron, the balance being substantially all aluminum.

2. A bearing metal alloy containing about 1-10% of lead, 1-10% of antimony, 0.1-3% of silicon, and 0.1-10% of nickel, the balance being substantially all aluminum.

3. A bearing metal alloy containing about 1-10% of lead, 1-10% of antimony, 0.1-3% of silicon and 0.1-10% of cobalt, the balance being substantially all aluminum.

4. A bearing metal alloy containing about 1-10% of lead, 1-10% of antimony, 0.1-3% of silicon, and 0.1-10% of iron, the balance being substantially all aluminum.

EUGEN VADERS.